

# United States Patent [19]

Anceschi et al.

[11] Patent Number: 5,051,111

[45] Date of Patent: Sep. 24, 1991

[54] WHITENER DISPERSION

[75] Inventors: **Italo Anceschi, Muttenz; Werner Fringeli, Laufen, both of Switzerland; Martin Jöllenbeck, Solingen, Fed. Rep. of Germany; Georges Mahler, Mulhouse, France; Willy Schürings, Grenzach-Wyhlen, Fed. Rep. of Germany**

[73] Assignee: **Ciba-Geigy Corporation, Ardsley, N.Y.**

[21] Appl. No.: 275,231

[22] Filed: Nov. 22, 1988

[30] Foreign Application Priority Data

Nov. 27, 1987 [CH] Switzerland 4630/87

[51] Int. Cl.<sup>5</sup> C09B 57/00; C09K 11/04

[52] U.S. Cl. 8/648; 252/301.21; 252/301.22; 252/310.23; 252/301.24; 8/922

[58] Field of Search 252/301.21, 301.22, 252/301.23, 301.24; 8/922, 553, 648

[56] References Cited

U.S. PATENT DOCUMENTS

3,575,866 4/1971 Strobel et al. 252/301.29  
3,928,329 12/1975 Fleck et al. 252/301.24  
4,070,319 1/1978 Carel et al. 252/301.21  
4,212,763 7/1980 Fringel 252/301.23

4,231,741 11/1980 Gunther et al. 252/301.23  
4,316,815 2/1982 Mercer et al. 252/301.22  
4,330,427 5/1982 Martini et al. 252/301.24  
4,336,155 6/1982 Martini et al. 252/301.23  
4,363,744 12/1982 Gunther et al. 252/301.24  
4,400,294 8/1983 Martini et al. 252/301.24  
4,416,795 11/1983 Martini et al. 252/301.24  
4,605,511 8/1986 Fringel 252/301.23  
4,666,627 5/1987 Meyer 252/301.22  
4,717,502 1/1988 Schmid 252/301.23

## OTHER PUBLICATIONS

European Search Report, 88 81 0794.

Primary Examiner—John F. Niebling

Assistant Examiner—Steven P. Marquis

Attorney, Agent, or Firm—George R. Dohmann; Edward McC. Roberts

[57] ABSTRACT

There are disclosed aqueous dispersions comprising water-insoluble or sparingly soluble fluorescent whitening agents, water-soluble fluorescent whitening agents, dispersants, optional solubilizers, further optional assistants and a copolymer of 2-vinylpyrrolidone and 3-vinylpropionic acid, their preparation and the use thereof for whitening polyester/cellulose fiber material. These novel dispersions are storage-stable and temperature-stable.

23 Claims, No Drawings

## WHITENER DISPERSION

The present invention relates to an aqueous whitener dispersion and to the preparation thereof, as well as to the use of said dispersion for whitening polyester/cellulose blends.

The novel whitener dispersion is stable in the temperature range up to 40° C. and storage-stable for up to six months and is able to whiten the polyester component and the cellulose component of polyester/cellulose blends simultaneously in one application step, and produces excellent white effects on the treated material.

Accordingly, the present invention relates to a novel aqueous dispersion comprising at least one water-insoluble or sparingly soluble fluorescent whitening agent, an optional solubiliser, at least one anionic, cationic and/or non-ionic surfactant, and further optional assistants, which dispersion additionally comprises a copolymer of 2-vinylpyrrolidone and 3-vinylpropionic acid.

5 cent whitening agent, 4-20% of water-soluble fluorescent whitening agent, 2-20% of dispersant, 5-25% of solubiliser, 1-20% of copolymer of 2-vinylpyrrolidone and 3-vinylpropionic acid, and 0.1-10% of further assistants.

In the present context and throughout this specification, percentages are by weight.

Particularly preferred dispersions comprise 5-10% of water-insoluble or sparingly soluble fluorescent whitening agent, 4-10% of water-soluble fluorescent whitening agent, 2-5% of dispersant, 10-25% of solubiliser, 3-6% of copolymer of 2-vinylpyrrolidone and 3-vinylpropionic acid, and 0.1-5% of further assistants.

10 The water-insoluble or sparingly soluble whitening agents are compounds or mixtures of compounds, for example of the class of the stilbenes, distyrylbenzenes, diphenylbistyrils, triazinyls, benzoxazoles, bis(benzoxazoles), bis(benzoxazolyl)thiophenes, bis(benzoxazolyl)naphthalenes, pyrenes, coumarins and naphthalene-peridicarboximides. Preferred compounds are 15 those of formulae:



The dispersion of this invention preferably comprises 3-20% of water-insoluble or sparingly soluble fluores-

wherein

3

A = 2-benzoxazolyl,  $-\text{CH}=\text{CH}-\text{CN}$ ,  $-\text{CH}=-$   
 $\text{CH}-\text{COOR}_2$ ,  $-\text{COOR}_2$  or halogen,  
 B = phenyl if A is 2-benzoxazolyl,  
 B =  $-\text{CH}=\text{CH}-\text{CN}$  if A is  $-\text{CH}=\text{CH}-\text{CN}$ ,  
 B =  $-\text{CH}=\text{CH}-\text{COOR}_2$  if A is  $-\text{CH}=-$   
 $\text{CH}-\text{COOR}_2$ ,  
 B = 2-benzoxazolyl if A is  $-\text{COOR}_2$ ,  
 B = naphthalene-triazolyl if A is halogen or  $-\text{COOR}_2$ ,  
 B = 1,2,4-oxadiazole if A is 2-benzoxazolyl, and  
 R = H,  $\text{C}_1\text{-C}_4$ alkyl,  
 $\text{R}_1 = \text{H, C}_1\text{-C}_4$ alkyl and CN,  
 $\text{R}_2 = \text{C}_1\text{-C}_4$ alkyl,  
 10

4

$R_5 = C_1-C_4$  alkyl or phenyl,  
 $X = C, N$   
 $Y = \text{phenyl or a radical of formula}$



10 and  
 $n=0-2$

Particularly interesting compounds are those of formulae:



(7)



(8)



(9)



(10)



(11)



(12)

-continued

(13)



(14)



(15)



(16)



(17)



wherein M=Li, Na, K



(18)

55

-continued

R3 = —NH—

, and

R4 = —N

60

65 and M=Li, Na, K or ammonium as well as the mixtures I to VI:

wherein





80%



20%



80%



20%



27%



13%



60%



20% or 40%



80% or 60%



40%

-continued



The water-soluble fluorescent whitening agents are compounds or mixtures of compounds of the class, for example, of the bis(triazinyl)diaminostilbenes, distyryl biphenyls and triazolylstilbenes, such as the compounds

30 diethylene glycol, propylene glycol, aminoethanesulfonic acid or salts thereof, ethanolaminopropionamide, cyanoethylbenzylamine, cyanoethylmethanolamine, M' is H, Li, Na, K, ammonium or C<sub>1</sub>-C<sub>4</sub>alkylammonium;



of formulae

wherein X<sub>1</sub> and X<sub>1</sub>' are H or Cl and M'' is H, ammonium



wherein X and X' are aniline, aniline-3-sulfonic acid, aniline-4-sulfonic acid, aniline-2,5-disulfonic acid or

or C<sub>1</sub>-C<sub>4</sub>alkylammonium and, where appropriate, Li, Na or K;



salt thereof or methanol, Y' and Y'' are aniline, ethanolamine, diethanolamine, N-methylethanolamine, diisopropanolamine, ethylamine, diethylamine, morpholine,

wherein X<sub>2</sub> and X<sub>2</sub>' are H, SO<sub>3</sub>M and M is Li, Na, K, ammonium or C<sub>1</sub>-C<sub>4</sub>alkylammonium.

Especially preferred are combinations of compounds of formula (19) with compounds of formula (3) and/or (5), as well as with the mixtures II, III, V and/or VI.

The ratio of water-soluble to water-insoluble or sparingly soluble fluorescent whitening agents is governed by the ratio of polyester:cellulose of the polyester/cellulose blends to be whitened. In general, 0.15–0.25% of water-soluble fluorescent whitening agent per 100% of cellulose, and 0.15–0.25% of water-insoluble or sparingly soluble fluorescent whitening agent per 100% of polyester, will be used.

The cationic, anionic and/or non-ionic dispersants are the customary dispersants for water-insoluble or sparingly soluble fluorescent whitening agents.

Examples of anionic suitable dispersants are condensates of aromatic sulfonic acids with formaldehyde as well as ligninsulfonates. Particularly suitable anionic dispersants are condensates of formaldehyde with naphthalenesulfonic acid as well as dihexylsulfosuccinates.

Suitable cationic dispersants are, for example, quaternary fatty amine polyglycol ethers.

It is preferred, however, to use non-ionic dispersants, for example: ethylene oxide adducts of the class of adducts of ethylene oxide with higher fatty acids, saturated or unsaturated fatty alcohols, mercaptans, fatty acid amides, fatty acid alkylolamides or fatty amines, or with alkylphenols or alkylthiophenols in which the alkyl moiety contains at least 7 carbon atoms, which adducts contain preferably 5 to 100 mol of ethylene oxide per 1 mol of the cited compounds, as well as block polymers of ethylene oxide and propylene oxide. Individual ethylene oxide units can be replaced by other epoxides, for example styrene oxide or, preferably, propylene oxide.

Representative individual ethylene oxide adducts are:

a) adducts of saturated and/or unsaturated C<sub>8</sub>–C<sub>2</sub> of fatty alcohols with 5 to 100 mol of ethylene oxide per mol of alcohol, preferably of saturated linear C<sub>16</sub>–C<sub>18</sub> alcohols with 10 to 80 mol, preferably 25 mol, of ethylene oxide per mol of alcohol;

b) adducts of saturated and/or unsaturated C<sub>8</sub>–C<sub>2</sub> of fatty acids with 5 to 20 mol of ethylene oxide per mol of acid, preferably ethoxylated castor oil;

c) adducts of alkylphenols containing 7 to 12 carbon atoms in the alkyl moiety with 5 to 25 mol of ethylene oxide per mol of phenolic hydroxy group, preferably of mono- or dialkylphenols with 10 to 20 mol of ethylene oxide per mol of phenolic hydroxy group;

d) adducts of saturated and/or unsaturated C<sub>8</sub>–C<sub>2</sub> of fatty acid amides with 5 to 20 mol of ethylene oxide per mol of acid amide, preferably of oleylamides with 8 to 15 mol of ethylene oxide per mol of acid amide;

e) adducts of saturated and/or unsaturated C<sub>8</sub>–C<sub>2</sub> of fatty amines with 5 to 20 mol of ethylene oxide per mol of amine, preferably of oleylamines with 8 to 15 mol of ethylene oxide per mol of amine;

f) block polymers of ethylene oxide and propylene oxide with 10–80% of ethylene oxide and having molecular weights of 1000 to 80 000;

g) polyadducts of ethylene oxide and propylene oxide with ethylenediamine.

The adducts cited in a) to f) are preferred. It is also possible to use mixtures of the adducts of a) to g) with one another.

By solubilisers, which are used especially for the water-soluble fluorescent whitening agents, are meant hydroscopic agents such as polyethylene glycols preferably having molecular weights in the range from 200 to

40 000, most preferably from 1000 to 6000, as well as urea, tetramethylurea, triethanolamine, diethylene glycol, propylene glycol, cumenesulfonates, xenesulfonates and benzenesulfonates, monoethylene, diethylene and polyethylene glycol monoethyl and diethyl ester and monoethylene, diethylene and polyethylene glycol ether acetates.

It is further very advantageous that the dispersant as well as the solubiliser should be compatible with the whitener dispersion, i.e. that no precipitation results and that homogeneous dispersions are obtained.

The dispersion of this invention may also contain further assistants, for example textile auxiliaries, shading dyes, foam inhibitors and, especially, anti-freeze agents such as polyols, preferably di- or polyalcohols such as ethylene glycol, propylene glycol, diethylene glycol, glycerol and/or sorbitol, humectants, surfactants, for example polyethylene glycols having molecular weights in the range from 200 to 6 000, and/or microbicides such as chloroacetamide or aqueous formaldehyde solutions, as well as fungicides.

The salient feature of the invention is that the whitener dispersion contains a copolymer of 2-vinylpyrrolidone and 3-vinylpropionic acid. Such copolymers are known and can be prepared by known methods.

A particularly preferred whitener dispersion comprises 5–10% of water-insoluble or sparingly soluble fluorescent whitening agent of the class of the bis(benzoxazolyl)thiophenes, 4–10% of water-soluble fluorescent whitening agent of the class of the bis(triazinyl)-diaminostilbenedisulfonic acids, 2–5% of ethoxylated C<sub>16</sub>–C<sub>18</sub> fatty alcohol or ethylene oxide/propylene oxide block polymer as dispersant, 3–6% of copolymer of 2-vinylpyrrolidone and 3-vinylpropionic acid, and 14–16% of polyethylene glycol or 10–25% of urea as solubiliser, 0–0.5% of shading dye and 0.1–0.5% of formaldehyde as further assistants.

The whitener dispersion of this invention is prepared, for example, a) by mixing the separately prepared and formulated individual components—the separately formulated water-insoluble or sparingly soluble fluorescent whitening agent and the separately formulated water-soluble fluorescent whitening agent are preferably mixed—or b) by jointly formulating the individual components, for example by grinding in a microsol mill, bead mill, sand mill or dynamill to a particle size smaller than 5 μm.

The novel dispersions are used in particular for whitening polyester/cellulose fibre material, preferably polyester/cotton fabric, by applying said dispersions by a single step method to the material. In this context, "single step" means that the water-insoluble or sparingly soluble fluorescent whitening agent is applied simultaneously with the water-soluble fluorescent whitening agent. Application is made preferably by the exhaust process or also by the pad process, in weakly acid to strongly alkaline medium. A particular advantage of this process is that the polyester component and the cellulose component of the material are simultaneously whitened.

The invention is illustrated by the following non-limitative Examples, in which parts and percentages are by weight.

#### EXAMPLE 1

15 parts of a mixture of 60% of the sparingly soluble fluorescent whitening agent of formula

and 57% of the water-soluble fluorescent whitening agent of formula



and 40% of the water-soluble fluorescent whitening agent of formula

2.0 parts of the adduct of a C<sub>16</sub>-C<sub>18</sub>fatty alcohol with 25 mol of ethylene oxide,  
20.0 parts of polyethylene glycol 4000,  
0.5 part of 37% formaldehyde,  
10.0 parts of a 30% aqueous copolymer of 2-vinylpyrrolidone and 3-vinylpropionic acid, and  
49.5 parts of water are ground in a stirred ball mill with glass beads until the dispersion has a particle



2.0 parts of the adduct of a C<sub>16</sub>-C<sub>18</sub>fatty alcohol with 25 mol of ethylene oxide,  
15.0 parts of polyethylene glycol 4000,  
0.3 part of an anthraquinone dye,  
0.5 part of 37% formaldehyde,  
14.0 parts of a 30% aqueous copolymer of 2-vinylpyrrolidone and 3-vinylpropionic acid, and  
53.2 parts of water are ground in a stirred ball mill with glass beads until the dispersion has a particle size of less than 2  $\mu$ m. The glass beads are then separated, affording a homogeneous, readily pourable and pumpable liquid formulation having a 15% content of fluorescent whitening agent. The dispersion is storage-stable for several months at room temperature as well as at 40° C.

#### EXAMPLE 2

18 parts of a mixture of 43% of the sparingly soluble fluorescent whitening agent of formula



60

65

size of less than 2  $\mu$ m. The glass beads are then separated, affording a homogeneous, readily pourable and pumpable liquid formulation having a 15% content of fluorescent whitening agent. The dispersion is storage-stable for several months at room temperature as well as at 40° C.

#### EXAMPLE 3

15 parts of a mixture of 60% of the sparingly soluble fluorescent whitening agent of formula



and 40% of the water-soluble fluorescent whitening agent of formula



15

2.0 parts of an ethylene oxide/propylene oxide block polymer with 80% of ethylene oxide and having a molecular weight of ca. 16 000,  
 15.0 parts of urea,  
 0.3 part of an anthraquinone dye,  
 0.5 part of 37% formaldehyde,  
 14.0 parts of a 30% aqueous copolymer of 2-vinylpyrrolidone and 3-vinylpropionic acid, and  
 53.2 parts of water are ground in a stirred ball mill with glass beads until the dispersion has a particle size of less than 2  $\mu$ m. The glass beads are then separated, affording a homogeneous, readily pourable and pumpable liquid formulation having a 15% content of fluorescent whitening agent. The dispersion is storage-stable for several months at room temperature as well as at 40° C.

25

35

2 parts of an ethylene oxide/propylene oxide block polymer with 10% of ethylene oxide and having a molecular weight of ca. 1060,  
 15 parts of urea,

0.3 part of an anthraquinone dye,  
 0.5 part of 37% formaldehyde,  
 14 parts of a 30% aqueous copolymer of 2-vinylpyrrolidone and 3-vinylpropionic acid, and  
 53.2 parts of water are ground in a stirred ball mill with glass beads until the dispersion has a particle size of less than 2  $\mu$ m. The glass beads are then separated, affording a homogeneous, readily pourable and pumpable liquid formulation having a 15% content of fluorescent whitening agent. The dispersion is storage-stable for several months at room temperature as well as at 40° C.

## EXAMPLE 4

15 parts of a mixture of 60% of the sparingly soluble fluorescent whitening agent of formula

40



45

and 40% of the water-soluble fluorescent whitening agent of formula

15 parts of a mixture of 60% of the sparingly soluble fluorescent whitening agent of formula

## EXAMPLE 5

and 40% of the water-soluble fluorescent whitening agent of formula





Z = Na, diethanolamine (2:1)

2 parts of an adduct of a C<sub>16</sub>-C<sub>18</sub> fatty alcohol with 25 mol of ethylene oxide. 25

15 parts of polyethylene glycol 5-6000,

3.3 parts of ethylene glycol,

0.5 part of 37% formaldehyde,

14 parts of a 30% aqueous copolymer of 2-vinylpyrrolidone and 3-vinylpropionic acid, and 30

50.2 parts of water are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C. 35

**EXAMPLE 6**

9.20 parts of the sparingly soluble fluorescent whitening agent of formula

- 2 parts of the adduct of a C<sub>16</sub>-C<sub>18</sub> fatty alcohol with 25 mol of ethylene oxide,
- 15 parts of polyethylene glycol 4000,
- 0.5 part of 37% formaldehyde,
- 14.0 parts of a 30% aqueous copolymer of 2-vinylpyrrolidone and 3-vinylpropionic acid, and
- 52.36 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C.

### EXAMPLE 7

40 7.9 parts of the sparingly soluble fluorescent whitening agent of formula



(active content 98%)



(active content 98%)

and 6.64 of the water-soluble fluorescent whitening agent of formula

and 11.4 parts of the water-soluble fluorescent whitening agent of formula





Y,Y' =  $\text{N}(\text{CH}_2\text{CH}_2\text{OH})_2$

(active content 90%)

2 parts of an adduct of a C<sub>16</sub>-C<sub>18</sub> fatty alcohol and 25 mol of ethylene oxide,  
20 parts of polyethylene glycol 4000,  
0.2 part of chloroacetamide,  
10 parts of a 30% aqueous copolymer of 2-vinylpyrrolidone and 3-vinylpropionic acid, and  
48.5 parts of water are ground in a stirred ball mill 20 with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C.

#### EXAMPLE 8

9.20 parts of the sparingly soluble fluorescent whitening agent of formula 30



(active content 98%)

40

2.0 parts of an adduct of a C<sub>16</sub>-C<sub>18</sub> fatty alcohol and 25 mol of ethylene oxide,  
15.0 parts of polyethylene glycol 4000,  
0.2 part of chloroacetamide,  
14.0 parts of a 30% aqueous copolymer of 2-vinylpyrrolidone and 3-vinylpropionic acid, and  
52.96 parts of water are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C.

#### EXAMPLE 9

9.20 parts of the sparingly soluble fluorescent whitening agent of formula



(active content 98%)

and 6.64 parts of the water-soluble fluorescent whitening agent of formula

and 6.64 parts of the water-soluble fluorescent whitening agent of formula



Y,Y' =  $\text{N}(\text{CH}_2\text{CH}_2\text{OH})_2$

(active content 90%)



Y,Y' =  $\text{N}(\text{CH}_2\text{CH}_2\text{OH})_2$

(active content 90%)

## 21

2.0 parts of an ethylen oxide/propylene oxide block polymer with 80% of ethylene oxide and having a molecular weight of ca. 16 000,  
 15.0 parts of urea,  
 0.2 part of chloroacetamide,  
 14.0 parts of a 30% aqueous copolymer of 2-vinylpyrrolidone and 3-vinylpropionic acid, and  
 52.96 parts of water are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C. 15

## EXAMPLE 10

9.20 parts of the sparingly soluble fluorescent whitening agent of formula 20



(active content 98%)

and 6.64 parts of the water-soluble fluorescent whitening agent of formula

2.0 parts of an ethylene oxide/propylene oxide block polymer with 80% of ethylene oxide and having a molecular weight of ca. 1060,  
 15.0 parts of urea,  
 0.2 parts of chloroacetamide,  
 14.0 parts of a 30% aqueous copolymer of 2-vinylpyrrolidone and 3-vinylpropionic acid, and  
 52.96 parts of water are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C. 15

## 22

2.0 parts of an ethylene oxide/propylene oxide block polymer with 80% of ethylene oxide and having a molecular weight of ca. 1060,  
 15.0 parts of urea,  
 0.2 parts of chloroacetamide,  
 14.0 parts of a 30% aqueous copolymer of 2-vinylpyrrolidone and 3-vinylpropionic acid, and  
 52.96 parts of water are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C.

## EXAMPLE 11

5.30 parts of the sparingly soluble fluorescent whitening agent of formula 20



(active content 98%)

and 13.24 parts of the water-soluble fluorescent whitening agent of formula



(active content 74%)

2.0 parts of the adduct of a C<sub>16</sub>-C<sub>18</sub>fatty alcohol with 5  
25 mol of ethylene oxide,  
20.0 parts of polyethylene glycol 4000,  
0.2 part of chloroacetamide,  
14.0 parts of a 30% aqueous copolymer of 2-vinylpyr-  
olidone and 3-vinylpropionic acid, and  
54.74 parts of water are ground in a stirred ball mill 10  
with glass beads until the dispersion has a particle  
size of less than 2  $\mu\text{m}$ . The glass beads are then  
separated, affording a homogeneous, readily pour-  
able and pumpable liquid formulation having a 15% 15  
content of fluorescent whitening agent. The  
dispersion is storage-stable for several months at  
room temperature as well as at 40° C.

## EXAMPLE 12

8.16 parts of the sparingly soluble fluorescent whiten- 20  
ing agent of formula



(active content 98%)

and 8.97 parts of the water-soluble fluorescent whiten-  
ing agent of formula

X, X' =  $-\text{NH}-\text{C}_6\text{H}_4-\text{SO}_3\text{Na}$ Y, Y' =  $\text{NH}-\text{CH}_2\text{CH}_2\text{OH}$ 

(active content 78%)

2.0 parts of the adduct of a C<sub>16</sub>-C<sub>18</sub>fatty alcohol with 50  
25 mol of ethylene oxide,  
20.0 parts of polyethylene glycol 4000,  
0.2 part of chloroacetamide,  
14.0 parts of a 30% aqueous copolymer of 2-vinylpyr-  
olidone and 3-vinylpropionic acid, and  
46.47 parts of water are ground in a stirred ball mill 55  
with glass beads until the dispersion has a particle  
size of less than 2  $\mu\text{m}$ . The glass beads are then

-continued

separated, affording a homogeneous, readily pour-  
able and pumpable liquid formulation having a  
15% content of fluorescent whitening agent. The  
dispersion is storage-stable for several months at  
room temperature as well as at 40° C.

## EXAMPLE 13

8.25 parts of the sparingly soluble fluorescent whiten- 20  
ing agent of formula



(active content 100%)

1.45 parts of the sparingly soluble fluorescent whitening  
agent of formula



(active content 100%)

5.90 parts of the water-soluble fluorescent whitening  
agent of formula



-continued



Y, Y' =  $\text{N}(\text{CH}_2\text{CH}_2\text{OH})_2$   
(active content 90%)

10

2.0 parts of the adduct of a C<sub>16</sub>-C<sub>18</sub> fatty alcohol with 25 mol of ethylene oxide,  
2.5 parts of 1,2-propylene glycol,  
0.5 part of a modified aldehyde/ketone condensation resin,  
16.0 parts of polyethylene glycol 4000,  
0.2 part of chloroacetamide,  
14.0 parts of a 30% aqueous copolymer of 2-vinylpyrrolidone and 3-vinylpropionic acid, and  
49.26 parts of water, are ground in a stirred ball mill 20 with glass beads until the dispersion has a particle size of less than 2  $\mu\text{m}$ . The glass beads are then separated, affording a homogeneous, readily pourable and pumpable liquid formulation having a 15% content of fluorescent whitening agent. The 25 dispersion is storage-stable for several months at

15



(active content 100%)

7.05 parts of the water-soluble fluorescent whitening agent of formula



Y, Y' =  $\text{N}(\text{CH}_2\text{CH}_2\text{OH})_2$   
(active content 90%)

room temperature as well as at 40° C.

## EXAMPLE 14

8.08 parts of the sparingly soluble fluorescent whitening agent of formula 55



(active content 100%)

60

65

1.42 parts of the sparingly soluble fluorescent whitening agent of formula

2.0 parts of the adduct of a C<sub>16</sub>-C<sub>18</sub> fatty alcohol with 25 mol of ethylene oxide,  
2.5 parts of 1,2-propylene glycol,  
0.5 part of a modified aldehyde/ketone condensation resin,  
8.0 parts of polyethylene glycol 4000,  
0.2 part of chloroacetamide,  
14.0 parts of a 30% aqueous copolymer of 2-vinylpyrrolidone and 3-vinylpropionic acid, and  
56.25 parts of water, are ground in a stirred ball mill 50 with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage stable for several months at room temperature as well as at 40° C.

## EXAMPLE 15

5.7 parts of the sparingly soluble fluorescent whitening agent of formula



5

(active content 100%)

1.0 part of the sparingly soluble fluorescent whitening agent of formula



(active content 100%)

25

## 11.2 parts of the water-soluble fluorescent whitening agent of formula



(active content 100%)

20 1.42 parts of the sparingly soluble fluorescent whitening agent of formula



2.0 parts of the adduct of a C<sub>16</sub>-C<sub>18</sub> fatty alcohol with 25 mol of ethylene oxide,

1.75 parts of 1,2-propylene glycol,

0.35 part of a modified aldehyde/ketone condensation resin,

15.0 parts of polyethylene glycol,

0.2 part of chloroacetamide,

14.0 parts of a 30% aqueous copolymer of 2-vinylpyrrolidone and 3-vinylpropionic acid, and

48.8 parts of water, are ground in a stirred ball mill with glass beads until the dispersion has a particle

60



(active content 100%)

## 6.25 parts of the water-soluble fluorescent whitening agent of formula



(active content 88%)

2.0 parts of an adduct of a C<sub>16</sub>-C<sub>18</sub>fatty alcohol and  
25 mol of ethylene oxide,

2.5 parts of 1,2-propylene glycol,

0.5 part of a modified aldehyde/ketone condensation resin,

0.2 part of chloroacetamide,

14.0 parts of a 30% aqueous copolymer of 2-vinylpyrrolidone and 3-vinylpropionic acid, and

65.05 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage-stable for several months at room temperature as well as at 40° C.

30

35

-continued  
(active content 100%)

25 0.82 part of the sparingly soluble fluorescent whitening agent of formula



(active content 100%)

4.64 parts of the sparingly soluble fluorescent whitening agent of formula

40

6.25 parts of the water-soluble fluorescent whitening agent of formula



(active content 88.5%)



2.0 parts of the adduct of a C<sub>16</sub>-C<sub>18</sub>fatty alcohol with  
25 mol of ethylene oxide,

1.4 parts of 1,2-propylene glycol,

0.3 part of a modified aldehyde/ketone condensation resin,

50.0 parts of triethanolamine,

0.2 part of chloroacetamide,

31

14.0 parts of a 30% aqueous copolymer of 2-vinylpyrrolidone and 3-vinylpropionic acid, and  
 20.4 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 15% content of fluorescent whitening agent. The dispersion is storage stable for several months at room temperature as well as at 40° C.

10

## EXAMPLE 18

9.2 parts of the sparingly soluble fluorescent whitening agent of formula



(active content 98%)

9.0 parts of the sparingly soluble fluorescent whitening agent of formula

15

20

46.6 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 15.6% content of fluorescent whitening agent. The dispersion is storage-stable for several months at room temperature as well as at 40° C.

## EXAMPLE 19

4.24 parts of the sparingly soluble fluorescent whitening agent of formula



(active content 100%)

1.06 parts of the sparingly soluble fluorescent whitening agent of formula



(active content 74%)

Z = 2:1 Na, diethanol ammonium.

2.0 parts of the adduct of a C<sub>16</sub>-C<sub>18</sub>fatty alcohol with 25 mol of ethylene oxide,  
 0.7 part of diethanolamine,  
 3.3 parts of ethylene glycol,  
 15.0 parts of polyethylene glycol 5000-6000,  
 0.2 part of chloroacetamide,  
 14.0 parts of a 30% aqueous copolymer of 2-vinylpyrrolidone and 3-vinylpropionic acid, and

60

65



(active content 100%)

5.2 parts of the sparingly soluble fluorescent whitening agent of formula



(active content 90%)

2.0 parts of the adduct of a C<sub>16</sub>-C<sub>18</sub>fatty alcohol with 20

25 mol of ethylene oxide,

12.0 parts of polyethylene glycol 4000,

0.2 part of chloroacetamide,

14.0 parts of a 30% aqueous copolymer of 2-vinylpyrrolidone and 3-vinyl propionic acid, and

61.3 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 30 10% content of fluorescent whitening agent. The dispersion is storage-stable for several months at room temperature as well as at 40° C.

-continued

(active content 100%)

0.67 part of the sparingly soluble fluorescent whitening 25 agent of formula



(active content 100%)

35 9.0 parts of the sparingly soluble fluorescent whitening agent of formula



(active content 74%)

ing agent of formula



65 2.0 parts of the adduct of a C<sub>16</sub>-C<sub>18</sub>fatty alcohol with 25 mol of ethylene oxide,

12.0 parts of polyethylene glycol 4000,

0.2 part of chloroacetamide,

14.0 parts of a 30% aqueous copolymer of 2-vinylpyrrolidone and 3-vinyl propionic acid, and

59.45 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 10% content of fluorescent whitening agent. The dispersion is storage-stable for several months at room temperature as well as at 40° C.

## EXAMPLE 21

4.24 parts of the sparingly soluble fluorescent whitening agent of formula



1.06 parts of the sparingly soluble fluorescent whitening agent of formula



5.2 parts of the sparingly soluble fluorescent whitening agent of formula



2.0 parts of the adduct of a C<sub>16</sub>-C<sub>18</sub>fatty alcohol with 25 mol of ethylene oxide,  
12.0 parts of polyethylene glycol 4000,  
0.2 part of chloroacetamide,  
14.0 parts of a 30% aqueous copolymer of 2-vinylpyrrolidone and 3-vinyl propionic acid, and  
61.3 parts of water, are ground in a stirred ball mill with glass beads until the dispersion has a particle size of less than 2  $\mu\text{m}$ . The glass beads are then separated, affording a homogeneous, readily pourable and pumpable liquid formulation having a 10% content of fluorescent whitening agent. The dispersion is storage-stable for several months at room temperature as well as at 40° C.

## EXAMPLE 22

1 g of the whitener dispersion according to any one of Examples 1-21 is predispersed in 10 ml of warm water of 40° C. that contains 1 g/l of a non-ionic dispersant (Irgasol NA). This preliminary dispersion is added to the warm whitener bath of 40° C. that contains 100 g of prebleached polyester/cellulose fabric (50:50) and 1 g/l of a non-ionic dispersant (Irgasol NA). After a 10 minute preliminary running of the goods, the bath is heated to 110° C. over 30 minutes. The goods are left in the bath for a further 40 minutes at this temperature. The bath is then cooled and the goods are rinsed and dried, to give a uniformly whitened fabric with a high degree of whiteness.

## EXAMPLE 23

A whitener dispersion according to any one of Examples 1 to 4 and 6 to 21 is predispersed as in Example 22. 20 This preliminary dispersion is added to the warm whitener bath of 40° C. that contains 100 g of polyester/cellulose fabric (50:50), 1 g/l of a non-ionic dispersant (Irgasol NA) and the chemicals necessary for bleaching the fabric (5 ml/l of H<sub>2</sub>O<sub>2</sub>, 35% by weight, 0.5 ml/l of diethylenetriaminopentacetic acid and 1 g/l of 100% NaOH). Application is made as in Example 22, to give a uniformly whitened and bleached fabric with a high degree of whiteness.

What is claimed is:

30 1. An aqueous dispersion comprising at least one water-insoluble or sparingly soluble fluorescent whitening agent, at least one water-soluble fluorescent whitening agent, an optional solubiliser, at least one anionic, cationic or non-ionic dispersant and further optional assistants, which dispersion additionally comprises a



55 copolymer of 2-vinylpyrrolidone and 3-vinylpropionic acid.

2. A dispersion according to claim 1, which comprises 3-20% of water-insoluble or sparingly soluble fluorescent whitening agent, 4-20% of water-soluble fluorescent whitening agent, 2-20% of dispersant, 5-25% of solubiliser, 1-20% of copolymer of 2-vinylpyrrolidone and 3-vinylpropionic acid, and 0.1-10% of further assistants.

60 3. A dispersion according to claim 2, which comprises 5-10% of water-insoluble or sparingly soluble fluorescent whitening agent, 4-10% of water-soluble fluorescent whitening agent, 2-5% of dispersant, 10-25% of solubiliser, 3-6% of copolymer of 2-vinyl-

pyrrolidone and 3-vinylpropionic acid, and 0.1-5% of further assistants.

4. A dispersion according to claim 1, wherein the water-insoluble or sparingly soluble fluorescent whitening agents are compounds or mixtures of compounds selected from the group consisting of the class of the stilbenes, distyrylbenzenes, distyrylbiphenyls, triazinyls, benzoxazoles, bis(benzoxazoles), bis(benzoxazolyl)thiophenes, bis(benzoxazolyl)naphthalenes, pyrenes, coumarins and naphthalene-peridicarboximides, and the water-soluble fluorescent whitening agents are compounds or mixtures of compounds selected from the class consisting of bis(triazinyl)diaminostilbenes, distyrylbiphenyls and triazolylstilbenes.

5. A dispersion according to claim 4, which contains at least one compound of formula



as water-insoluble or sparingly soluble fluorescent whitening agent.

6. A dispersion according to claim 4, which contains at least one compound of formula



wherein

A=2-benzoxazolyl, —CH=CH—CN, —CH=CH—COOR<sub>2</sub>, —COOR<sub>2</sub> or halogen,

B=phenyl if A is 2-benzoxazolyl,

B=—CH=CH—CN if A is —CH=CH—CN,

B=—CH=CH—COOR<sub>2</sub> if A is —CH=CH—COOR<sub>2</sub>,

B=naphthalene-triazolyl if A is halogen or —COOR<sub>2</sub>,

B=1,2,4-oxadiazole if A is 2-benzoxazolyl, and

R=H, C<sub>1</sub>-C<sub>4</sub>alkyl,

R<sub>1</sub>=H, C<sub>1</sub>-C<sub>4</sub>alkyl and CN,

R<sub>2</sub>=C<sub>1</sub>-C<sub>4</sub>alkyl,

as water-insoluble or sparingly soluble fluorescent whitening agent.

7. A dispersion according to claim 4, wherein the water-insoluble or sparingly soluble fluorescent whitening agent is a compound of formula



wherein R<sub>2</sub> is C<sub>1</sub>-C<sub>4</sub>alkyl.

8. A dispersion according to claim 4, wherein the water-insoluble or sparingly soluble fluorescent whitening agent is a compound of formula



(4)

wherein R<sub>5</sub> is C<sub>1</sub>-C<sub>4</sub>alkyl or phenyl, and R is H or C<sub>1</sub>-C<sub>4</sub>alkyl, X<sub>1</sub> is C or N, and Y is phenyl or a radical of formula



9. A dispersion according to claim 4, wherein the water-insoluble or sparingly soluble fluorescent whitening agent is a compound of formula



(5)

wherein n is 0 to 2 and R<sub>2</sub> is C<sub>1</sub>-C<sub>4</sub>alkyl.

10. A dispersion according to claim 4, wherein the water-insoluble or sparingly soluble fluorescent whitening agent is a compound of formula



(6)

wherein R<sub>2</sub> is C<sub>1</sub>-C<sub>4</sub>alkyl.

11. A dispersion according to claim 4, wherein the water-insoluble or sparingly soluble fluorescent whitening agent is a compound of formula



(7)

12. A dispersion according to claim 4, wherein the water-insoluble or sparingly soluble fluorescent whitening agent is a compound of formula



wherein



10 wherein M is Li, Na or K.

14. A dispersion according to claim 4, wherein the water-soluble fluorescent whitening agent is a compound of formula



25 wherein X and X' are aniline, aniline-3-sulfonic acid, aniline-4-sulfonic acid, aniline-2,5-disulfonic acid or salts thereof or methanol, Y' and Y'' are aniline, ethanolamine, diethanolamine, N-methylethanolamine, diisopropanolamine, ethylamine, diethylamine, morpholine, diethylene glycol, propylene glycol, aminoethanesulfonic acid or salts thereof, ethanolaminopropionamide, cyanoethylbenzylamine, cyanoethylmethanolamine, and M' is H, Li, Na, K, ammonium or C<sub>1</sub>-C<sub>4</sub>alkylammonium.

15. A dispersion according to claim 4, wherein the water-soluble fluorescent whitening agent is a compound of formula



wherein X<sub>1</sub> and X<sub>1</sub>' are H or Cl and M'' is H, ammonium or C<sub>1</sub>-C<sub>4</sub>alkylammonium and, where appropriate, Li, Na or K.

and M is Na, Li, K or ammonium.

13. A dispersion according to claim 4, wherein the water-insoluble or sparingly soluble fluorescent whitening agent is a compound of formula

16. A dispersion according to claim 4, wherein the water-soluble fluorescent whitening agent is a compound of formula



wherein X<sub>2</sub> and X<sub>2</sub>' are H, SO<sub>3</sub>M and M is Li, Na, K, ammonium or C<sub>1</sub>-C<sub>4</sub>alkylammonium.

17. A dispersion according to claim 4, which comprises a mixture of a water-soluble compound of formula



wherein X and X' are aniline, aniline-3-sulfonic acid, aniline-4-sulfonic acid, aniline-2,5-disulfonic acid or salts thereof or methanol, Y' and Y'' are aniline, ethanolamine, diethanolamine, N-methylethanolamine, diiso-

wherein R<sub>2</sub> is C<sub>1</sub>-C<sub>4</sub>alkyl and n is 0 to 2.

18. A dispersion according to claim 4, which comprises a mixture of a water-soluble compound of formula



propanolamine, ethylamine, diethylamine, morpholine, diethylene glycol, propylene glycol, aminoethanesulfonic acid or salts thereof, ethanolaminopropionamide, cyanoethylbenzylamine, cyanoethylethanolamine, and M' is H, Li, Na, K, ammonium or C<sub>1</sub>-C<sub>4</sub>alkylammonium; a water insoluble compound of formula



and/or a compound of formula

30 30. A dispersion according to claim 4, which comprises a mixture of a water-soluble compound of formula



35 a compound of formula



19. A dispersion according to claim 4, which comprises a mixture of a water-soluble compound of formula



propanolamine, ethylamine, diethylamine, morpholine, diethylene glycol, propylene glycol, aminoethanesulfonic acid or salts thereof, ethanolamiopropionamide, cyanoethylbenzylamine, cyanoethylethanolamine, and M' is H, Li, Na, K, ammonium or C<sub>1</sub>-C<sub>4</sub>alkylammonium; a water-insoluble compound of formula



and a water-soluble compound of formula



and a compound of formula



20. A dispersion according to claim 4, which comprises a water-insoluble compound of formula

25 21. A dispersion according to claim 1, which comprises 5-10% of at least one water-insoluble or sparingly soluble fluorescent whitening agent selected from the class of the bis(benzoxazole)thiophenes, 4-10% of at least one water-soluble fluorescent whitening agent selected from the class of the bis(triazinyl)diaminostilbenedisulfonic acids, 2-5% of ethoxylated C<sub>16</sub>-C<sub>18</sub>fatty alcohol or ethylene oxide/propylene oxide block polymer as dispersant, 3-6% of a copolymer of 2-vinylpyrrolidone and 3-vinylpropionic acid, and 14-16% of polyethylene glycol or 10-25% of urea as solubiliser, 0-0.5% of shading dye and 0.1-0.5% of formaldehyde as further assistants.

30 22. A method for whitening polyester/cellulose fibre material, which comprises the step of applying an aqueous dispersion to the fibre material said dispersion comprising at least one water-insoluble or sparingly soluble fluorescent whitening agent, at least one water-soluble fluorescent whitening agent, an optional solubilizer, at least one anionic, cationic or non-ionic dispersant and further optional assistants, which dispersion additionally comprises a copolymer of 2-vinylpyrrolidone and 3-vinylpropionic acid.

35 23. The method of claim 22 carried out as a single step exhaust process.

\* \* \* \* \*